



US005401333A

**United States Patent** [19]

Ouyang et al.

[11] Patent Number: **5,401,333**[45] Date of Patent: **Mar. 28, 1995**

[54] **METHOD OF MONITORING DRIED-IN-PLACE NON-CHROME POLYACRYLAMIDE BASED TREATMENTS FOR ALUMINUM**

[75] Inventors: **Jiangbo Ouyang, Bensalem; William L. Harpel, Langhorne, both of Pa.**

[73] Assignee: **Betz Laboratories, Inc., Trevose, Pa.**

[21] Appl. No.: **213,414**

[22] Filed: **Mar. 15, 1994**

[51] Int. Cl.<sup>6</sup> ..... **C23C 22/77**

[52] U.S. Cl. ..... **148/241; 148/247;  
148/251**

[58] Field of Search ..... **148/241, 247, 251**

[56] **References Cited**

**U.S. PATENT DOCUMENTS**

4,136,073 1/1979 Muro et al. ..... 260/29.2

4,191,596 6/1990 Dollman et al. ..... 148/247  
5,122,202 6/1992 Dykstra ..... 148/247  
5,129,967 7/1992 Sander ..... 148/247  
5,158,622 10/1992 Reichgott et al. ..... 148/247

*Primary Examiner*—Sam Silverberg

*Attorney, Agent, or Firm*—Alexander D. Ricci; Steven D. Boyd

[57] **ABSTRACT**

A process for measuring the coating weight of a dried-in-place non-chromate polyacrylamide/surfactant based conversion coating is disclosed. An ammonium hexafluorotitanate tracer added to such a conversion coating was found to not adversely affect coating properties. The tracer was found to remain proportional to the polymer matrix when the coating was analyzed by X-ray fluorescence.

**1 Claim, 1 Drawing Sheet**



**Figure 1**



**METHOD OF MONITORING DRIED-IN-PLACE  
NON-CHROME POLYACRYLAMIDE BASED  
TREATMENTS FOR ALUMINUM**

**FIELD OF THE INVENTION**

The present invention relates generally to non-chromate coatings for metals. More particularly, the present invention relates to a method for monitoring the formation of a non-chromate conversion coating on aluminum and aluminum alloys. The method of the present invention provides a non-chromium coating for aluminum and aluminum alloys which yields excellent paint adhesion, corrosion resistance and boiling water performance which can be monitored by conventional X-ray fluorescence techniques.

**BACKGROUND OF THE INVENTION**

The purposes of the formation of a chromate conversion coating on the surface of aluminum are to provide corrosion resistance, improve adhesion of coatings and for aesthetic reasons. The conversion coating improves the adhesion of coating layers such as paints, inks, lacquers and plastic coatings. A chromate coating is typically provided by contacting aluminum with an aqueous composition containing hexavalent or trivalent chromium ions, phosphate ions and fluoride ions. Typical chromium or chromate conversion coatings exhibit visible coloration ranging from gold to brown.

Growing concerns exist regarding the pollution effects of chromate and phosphate discharged into rivers and waterways by such processes. Because of the high solubility and the strongly oxidizing character of hexavalent chromium ions, conventional chromate conversion coating processes require extensive waste treatment procedures to control their discharge.

Chromate-free conversion coatings are known in the art. For example, U.S. Pat. No. 4,191,596 which issued to Dollman et al. discloses a composition for coating aluminum which comprises a polyacrylic acid and  $H_2ZrF_6$ ,  $H_2TiF_6$  or  $H_2SiF_6$ . U.S. Pat. No. 4,921,552 which issued to Sander et al. discloses a dried-in-place, non-chromate coating for aluminum. The coating composition consists essentially of  $H_2ZrF_6$ , a water soluble acrylic acid and homopolymers thereof and hydrofluoric acid.

U.S. Pat. No. 4,136,072 which issued to Muro et al., discloses a composition and process for the pretreatment of aluminum surfaces using an aqueous acidic bath containing a stable organic film forming polymer and a soluble titanium compound. U.S. Pat. No. 5,158,622 which issued to Reichgott et al. discloses a dried-in-place conversion coating for metal surfaces such as aluminum and aluminum alloys which employs an aqueous solution of water soluble maleic or acrylic acid/allyl ether copolymers alone or with an acid.

Most non-chromate pretreatments generate transparent coatings on metal surfaces. Furthermore, the lack of chromate makes actual coating weight measurements difficult. The coating weight of a chromate-based coating can be determined relatively easily by chrome X-ray fluorescence or chemical stripping and chemical titration of the coating. Non-chromate coatings may or may not be easily analyzed depending upon the materials present in the coating. For example, anionic polyacrylamide alone or in combination with a nonionic surfac-

tant provides an effective aluminum pretreatment, however, such coatings are not readily analyzed.

**SUMMARY OF THE INVENTION**

5 The present invention provides a method of measuring the coating weight of a dried-in-place non-chromate polyacrylamide/surfactant based conversion coating. The method of the present invention involves the addition of an easily traced agent to a dried-in-place non-  
10 chromate conversion coating. The easily traced agent does not adversely affect the corrosion resistance or adhesion properties of the conversion coating. The easily traced agent is incorporated into the conversion coating treatment solution and remains proportional to the polymer matrix in the formed conversion coating. The present inventors discovered that ammonium hexafluorotitanate was readily soluble in a polyacrylamide/-  
15 surfactant based pretreatment solution; remained proportional to the polymer matrix in the dried-in-place conversion coating; did not adversely affect the properties of the conversion coating; and was easily measured by X-ray fluorescence.

20 As used herein, the term aluminum refers to aluminum as well as alloys of aluminum. In addition, it is believed that the method of the present invention would similarly effective in the treatment of other metals, galvanized metals and Galvalume®. Galvalume is a registered trademark of Bethlehem Steel Corporation for a zinc-aluminum galvanized steel.

**DESCRIPTION OF THE DRAWINGS**

FIG. 1 is a plot of Ti counts (60 second accumulation) in X-Ray fluorescence vs. treatment solution concentration in %,

**DESCRIPTION OF THE PREFERRED  
EMBODIMENTS**

30 The present inventors have discovered a method of tracing the coating weight of a polyacrylamide-based dried-in-place conversion coating for aluminum without adversely affecting the properties of the coating. A tracer material is added to the conversion coating treatment solution. When an aluminum surface is treated, an amount of the tracer proportional to the amount of the treatment solution applied becomes a part of the conversion coating. The amount of tracer in the conversion coating can be easily measured, as by X-Ray fluorescence, and a standard plot used to determine the concentration of treatment material in the treatment bath.

35 40 The tracer material of the present invention does not adversely affect the conversion coating properties. The tracer material does not adversely affect paint adhesion, corrosion resistance or boiling water performance. The tracer material of the present invention exhibited a linear response in a plot of X-Ray fluorescence intensity versus treatment bath concentration. The tracer material did not evidence any solubility problems such as cloudiness or gel formation in the treatment bath.

45 50 The tracer material of the present invention is ammonium hexafluorotitanate. The present inventors discovered that when ammonium hexafluorotitanate was incorporated into a polyacrylamide/surfactant based conversion coating treatment solution, tracing of titanium in the formed conversion coating was relatively easy. The addition of ammonium hexafluorotitanate did not result in any adverse effects on the adhesion properties or corrosion resistance of the conversion coating. These results were unexpected in that the addition of ammonium

nium hexafluorotitanate to other alkaline conversion coating treatments resulted in detrimental effects on the treatment solution. Also, when other titanium sources were incorporated into a polyacrylamide/surfactant based conversion coating solution problems of instability, non-linear response in X-Ray fluorescence testing or coating performance deterioration were noted.

The ammonium hexafluorotitanate tracer of the present invention is typically added to a polyacrylamide/surfactant based dried-in-place conversion coating treatment solution concentrate in concentrations ranging from about 0.1 to 10% by weight of the treatment solution. Preferably about 0.5% ammonium hexafluorotitanate is added. A typical polyacrylamide/surfactant based treatment solution concentrate can include from 0.05 to 20% polyacrylamide and from about 0.05 to 20% nonionic surfactant. The preferred polyacrylamide treatment concentrate comprises 1% anionic polyacrylamide of molecular weight 2,000 to 500,000 and 1% anionic surfactant. The acrylate/acrylamide ratio of the polymer molecule can range from 1:1 to 9:1.

The present invention will now be further described with reference to a number of specific examples which are to be regarded solely as illustrative and not as restricting the scope of the present invention.

In the following examples, the effects of the coating weight monitor on the treatment adhesion properties and corrosion resistance were evaluated with a variety of tests familiar to those skilled in the art. These tests included: "T-bend", the tendency for paint to disadhere from a 180° bend in the metal (0 T=perfect); "cross-hatch", the tendency of paint to disadhere from areas between closely spaced lines scribed through the paint; "T-bend/boiling DI water", the tendency for paint to crack or flower at a 180° bend in the metal after soaking in boiling DI water for 20 minutes (no paint cracking or flowering is considered a pass); "reverse impact/boiling DI water", the tendency for paint to disadhere from reverse impacted metal after boiling in DI water for 20 minutes; "acidic acid salt spray", per ASTM B-287 (10=perfect).

#### EXAMPLE 1

Various titanium sources were tested as tracers in a polyacrylamide/surfactant based pretreatment solution. Potassium hexafluorotitanate was found to have limited solubility in the treatment solution resulting in a non-linear response when analyzed by X-Ray fluorescence. A

mixture of lactic acid titanate chelate ammonium salt (Tyzor-LA available from E. I. DuPont de Nemours, Wilmington, Del.) in a polyacrylamide/surfactant based treatment solution generated intense titanium X-Ray fluorescence, however, the mixture became cloudy at 120° F. and particles formed which were suspended in the solution.

#### EXAMPLE 2

Ammonium hexafluorotitanate was tested as a tracer in a polyacrylamide/surfactant based pretreatment solution. The treatment was applied to Q Panel 3003 aluminum test panels. The test panels were cleaned with a commercial alkaline cleaner (Betz Kleen® 4004, available from Betz Laboratories, Inc., Trevose, Pa.), rinsed with ambient tap water, squeegeed and spin coated with various concentrations of a polyacrylamide/surfactant pretreatment. The pretreatment comprised various dilutions of a concentrate of 1% anionic polyacrylamide (weight average molecular weight 2,000 to 500,000, acrylate/acrylamide ratio 1:1 to 9:1) 1% anionic surfactant (Triton X - 100 available from Union Carbide) and 0.5% ammonium hexafluorotitanate. FIG. 1 is a plot of Ti counts (60 second accumulation) measured on a Portaspec (model 2501) X-ray spectrograph versus treatment solution concentration in DI water. The figure shows a linear relationship between concentration and Ti count as measured by X-Ray fluorescence.

#### EXAMPLE 3

The process described in Example 2 was used with a polyacrylamide/surfactant based pretreatment with and without ammonium hexafluorotitanate and Betz DC 1904, a chromium based pretreatment available from Betz Laboratories. Three polyester single coat paints were applied to the treated surfaces using a drawdown bar and cured according to the manufacturer's specifications. Table I summarizes the results showing that the polyacrylamide treatment with ammonium hexafluorotitanate tracer of the present invention provided comparable results to prior art chromium-based pretreatments. In Table I, Treatment A is Betz DC 1904, Treatment B is a polyacrylamide/surfactant based pretreatment without ammonium hexafluorotitanate and Treatment C is a solution in accordance with the present invention as described in

#### EXAMPLE 2.

TABLE I

PPG Polyester Paint

| Treatment              | TB* | TB/BW | RI | RI/BW | PENCIL | MEK | AASS (500 hr) |       |
|------------------------|-----|-------|----|-------|--------|-----|---------------|-------|
|                        |     |       |    |       |        |     | SCRIBE        | FIELD |
| 13.5% A                | 0T  | PASS  | 10 | 10    | 3H     | 100 | 9.5           | 10    |
| 10% B                  | 0T  | PASS  | 10 | 10    | 3H     | 100 | 10            | 10    |
| 10% C                  | 0T  | PASS  | 10 | 10    | 4H     | 100 | 10            | 10    |
| Lilly Polyester Paint  |     |       |    |       |        |     |               |       |
| 13.5% A                | 0T  | PASS  | 10 | 2     | 2H     | 100 | 8             | 8.5   |
| 10% B                  | 0T  | PASS  | 10 | 5     | 3H     | 100 | 9.5           | 9     |
| 10% C                  | 0T  | PASS  | 10 | 7     | 4H     | 100 | 8             | 8     |
| Morton Polyceram Paint |     |       |    |       |        |     |               |       |
| 13.5% A                | 1T  | PASS  | 10 | 10    | 3H     | 100 | 9.5           | 8     |
| 10% B                  | 1T  | PASS  | 10 | 10    | 4H     | 100 | 7             | 7     |
| 10% C                  | 1T  | PASS  | 10 | 10    | 4H     | 100 | 9.5           | 10    |

\*TB: T-Bend

TB/BW: T-bend/Boiling water

RI: Reverse Impact, impact force: 40 in-lbs.

RI/BW: Reverse Impact/Boiling water

AASS: Acetic Acid Salt Spray

## EXAMPLE 4

Tyzor-LA, in levels similar to Examples 1 to 3 above, was added to a polyacrylamide/surfactant based pre-treatment. The solution became cloudy and a precipitate formed at temperatures of 120° and 140° F.

Ammonium hexafluorotitanate was added to a non-chromate treatment solution comprising an anionic polyacrylamide copolymer, an inorganic silicate and an organofunctional silane. The treatment solution became 10 cloudy and gelled at room temperature overnight.

These examples show that the combination of a polyacrylamide pretreatment and ammonium hexafluorotitanate tracer is unique in providing a pretreatment for aluminum which provides excellent paint adhesion and corrosion resistance and in which the coating weight can be easily measured by X-Ray fluorescence.

While the present invention has been described with respect to particular embodiments thereof, it is apparent 20 that numerous other forms and modifications of the

invention will be obvious to those skilled in the art. The appended claims and this invention generally should be construed to cover all such obvious forms and modifications which are within the true scope and spirit of the present invention.

We claim:

1. A process for monitoring the coating weight of an anionic polyacrylamide/surfactant based aluminum treatment comprising:

- a. adding ammonium hexafluorotitanate in concentrations ranging from about 0.1 to 10% by weight of a treatment solution to an anionic polyacrylamide/surfactant based treatment solution;
- b. treating an aluminum surface with said combination;
- c. subjecting the treated surface to X-Ray fluorescence to detect titanate in the coating wherein titanate detected by X-Ray fluorescence is proportional to the coating weight.

\* \* \* \* \*

25

30

35

40

45

50

55

60

65